

H. F. CHAPPELL.  
METHOD OF CALCINING ALUNITE.  
APPLICATION FILED MAY 8, 1913.

1,089,109.

Patented Mar. 3, 1914.

3 SHEETS-SHEET 1.

*Fig. 1.*



H. F. CHAPPELL.  
METHOD OF CALCINING ALUNITE.  
APPLICATION FILED MAY 8, 1913.

1,089,109.

Patented Mar. 3, 1914.

3 SHEETS—SHEET 2.

Fig. 2.



**WITNESSES**

*C. O'Neill  
P. Quigley*

**INVENTOR:**

INVENTOR.  
Howard F. Chappell.

BY

BY  
Fenn, Davis & Goldthorpe  
ATTORNEYS.

H. F. CHAPPELL.  
METHOD OF CALCINING ALUNITE.  
APPLICATION FILED MAY 8, 1913.

1,089,109.

Patented Mar. 3, 1914.

3 SHEETS—SHEET 3.

Fig. 3.



Fig. 4.



WITNESSES

*C. J. Neill*  
*K. G. Clark*

Fig. 5.



INVENTOR:

*Howard F. Chappell,*  
BY  
*Levine, Davis & Goldsberry.*  
ATTORNEYS.

# UNITED STATES PATENT OFFICE.

HOWARD F. CHAPPELL, OF NEW YORK, N. Y.

## METHOD OF CALCINING ALUNITE.

1,069,109.

Specification of Letters Patent. Patented Mar. 3, 1914.

Application filed May 8, 1913. Serial No. 736,269.

To all whom it may concern:

Be it known that I, HOWARD F. CHAPPELL, a citizen of the United States, residing in the borough of Manhattan, city, county, and State of New York, have invented certain new and useful Improvements in Methods of Calcining Alunite; and I do hereby declare the following to be a full, clear, and exact description of the invention, such as will enable others skilled in the art to which it appertains to make and use the same.

Prior to the present invention, it has been customary to calcine alunite in heaps in the open air, or in kilns similar to those used for calcining lime, permitting the gases given off from the alunite to mix freely with the products from the combustion of the fuel. Thus, in the kiln method of calcining, all the gases evolved throughout the entire mass, together with the products of combustion of the fuel employed, are discharged from the top of the kiln in a state of admixture. This mixed volume of gases contains not only the sulfurous and sulfuric acids and their anhydrides, but also the fire gases and the watery vapors incident to the driving off of the moisture and water of composition of the alunite. It is extremely difficult, under these circumstances to absorb and render innocuous the sulfur gases, and it is not practicable to recover the sulfuric anhydrid in the form of fuming acid. Aside from these difficulties and disadvantages attendant upon the disposition of the sulfur gases, the calcining operation itself, as heretofore practised, has been lacking in uniformity of product, certainty as to the time factor involved, economy of fuel, and regularity of progression.

I have discovered that the calcining operation can be carried on to very great advantage over the former practice, if conducted in two stages, and also, when so divided into two stages, that the sulfurous and sulfuric acids and their anhydrides can be readily and economically recovered, the sulfuric anhydrid being recoverable in part by condensation and in part by absorption. The proportion of sulfurous anhydrid with respect to the sulfuric anhydrid and sulfuric acid evolved from the charge is also capable of being diminished, as will herein-after more fully appear.

In the first stage of the calcining operation, the alunite is calcined in direct contact with the fuel gases, the fresh charge being

retained in the furnace area in which the first stage of the operation is proceeding until fumes of sulfuric acid just begin to be perceptible in the exit gases. At this time, the temperature at that part of the initial portion of the charge which is ready to be transferred is about 600° C. This partly calcined alunite is then transferred into a retort or muffle, where it is heated out of contact with the fire gases, from the temperature of about 600° C. with which it enters the retort to from 900° C. to 1,000° C., and until such time as there is no further evolution of sulfur fumes. The completely calcined alunite will be found to have practically all of the alumina insoluble in water and practically all of the potash present as sulfate of potash.

The gases from the second stage of the calcining operation are drawn off separately from the gases of the first stage of the calcining operation and are devoid of admixture with the fire gases or with the water vapor given off from the charge of the first stage.

The second stage of the calcining operation is, as above indicated, conducted in a retort or muffle and by heat applied from without, that is to say, by heat transmitted through the walls of the muffle from the fire gases. In order to more effectually distribute the heat throughout the retort or muffle, I admit a regulated quantity of air, and, in order to preheat the air and at the same time to partly cool the fully calcined portion of the charge prior to its exit from the retort, I first pass the air through that portion of the charge which has been fully calcined and is about to be discharged from the muffle. This not only preheats the air and partially cools the calcined ore, but it also effects an economy in fuel because it causes a more intimate distribution of the heat throughout the entire body of the charge undergoing calcination. When it is desired to produce a weaker acid than fuming sulfuric acid, a regulated amount of steam, preferably preheated, and in the same manner as the air, is introduced into the muffle; or, by admitting regulated quantities of both air and steam, acid of intermediate strength can be obtained. When it is desired to make fuming acid, steam is excluded. The sulfuric acid and  $SO_3$  are recovered by condensation or by condensation and absorption, and the  $SO_2$ , free from the

presence of moisture, is particularly adapted for the making of sulfuric acid by the contact process. In any case, the quantity of sulfurous anhydrid present in the gases drawn off from the second stage of the calcining operation tends to considerable diminution relatively to the sulfuric anhydrid and sulfuric acid.

In the accompanying drawings, I have illustrated a furnace adapted for the practice of the invention upon a considerable commercial scale.

Figure 1 represents a longitudinal sectional view of such a furnace partly broken away midway of its length, so as to accommodate the view to the scale upon which the drawing is made; Fig. 2 represents a vertical transverse section thereof; Fig. 3 represents a horizontal transverse section and partial plan view; Figs. 4 and 5 represent, respectively, views taken at right angles to each other and illustrating the discharge end of one of the upright muffles.

Similar letters of reference indicate similar parts throughout the several views.

Referring to the drawings A indicates a bench or fire chamber within which are located a series of upright retorts or muffles *a*, which may, conveniently, be twelve in number, as indicated in Fig. 3. These retorts are similar to those used for the gasification of coal, and they may conveniently be heated from three producers *B*, having flues *b* which discharge below the lowermost bench floor *C*. The bench is provided with a series of such floors, one above the other, with an intervening space, and these floors are provided with appropriate openings so as to give the gases a zig-zag course in rising through the fire chamber. This is readily effected, for instance, by permitting the gases to rise through openings near the side walls of the fire chamber in alternate floors and through middle openings in the intermediate floors, as indicated by the arrows in Fig. 2. The floors, as shown, may be readily supported upon projections on the outer sides of the retorts and like projections from the inner side walls of the fire chamber. At their upper ends, the retorts *a* open into perpendicular shafts *d* of the same interior cross-sectional dimensions as the retort and of approximately the same length. It will be further noted that the fire gases which have been used for heating the retorts or muffles, likewise enter the perpendicular shafts *d* referred to, and pass from their points of entrance at the bottom of the shafts *d* upward through the charge contained therein finally making their exit through the exit chimneys or flues *e*. These flues *e* are provided with regulating dampers *f* adapted to be automatically governed by any suitable intermediate mechanism, if desired, from a pyrometer *g*. I have merely

illustrated the intermediate mechanism diagrammatically, inasmuch as available constructions for this purpose are well known and do not require specific illustration and description.

The shafts *d* are adapted to be charged from suitable hoppers *h* having regulating gates *h'* as shown, and the hoppers may be charged conveniently from suitable elevators or otherwise. It is likewise convenient and desirable to have a single hopper feed a number of retorts, as indicated, for instance, in Fig. 1. To facilitate the draft, the exit flues *e* may be provided with an exhaust fan (not shown).

Each of the retorts discharges at its bottom into a water-jacketed casing *i*, which may be made up of two sections as shown more fully in Figs. 4 and 5, having a water inlet at *i'* and a water exit at *i''*, the sections being connected by a communicating pipe *i''*. These water cooled casings serve to regulate the temperature of the calcined product on its way to the discharge chute *C*, which is inclined laterally, so as to sustain the main weight of the charge, thereby appropriately relieving the weight that would otherwise be imposed upon the discharge gate *j*. Below the discharge gate *j* is located a swinging weighted valve *k*, whose function is to prevent steam generated from the calcined product as it falls into the water receptacle *D* from entering the bottom of the retorts. The receptacle *D* is provided with an inclined bottom and a water level is maintained, as indicated, with a suitable overflow pipe *l* leading into a tank *E* from which the material collected can be withdrawn by a pump *F*, or otherwise. An elevating screw conveyer *G* lifts the quenched calcined product and discharges it into a suitable receptacle. Each of the water-jacketed casings is provided with a tube *p* through which suitable test samples may be withdrawn from time to time, if desired.

At the bottom of each of the casings into which the retorts are discharged are located two pipes, one of which as *m* serves for the admission of air and the other, as *n*, serves for the admission of steam, both of these pipes being provided with regulating valves so as to permit the air and steam to be admitted in regulated amount. The air or steam passes through the completely calcined alunite and becomes highly preheated before entering the retort proper, thereby making available the heat of the calcined alunite for use in the interior of the retorts, thus supplementing the heat imparted from without by the fire gases. Furthermore, as the upward passage of the air or steam, as the case may be, facilitates the removal of the gases from the retorts and greatly decreases the fuel consumption.

Immediately above the tops of the re-

torts, exit pipes H are provided for the purpose of removing the gases generated in the retorts. Immediately above these pipes and on opposite sides of the shaft, but below the flues which lead into the shafts d are located pipes I, provided with valves. These pipes I are used to admit air or other aeriform fluid under pressure. This air, when properly regulated, prevents the fire gases which heat the retorts from entering the retorts, inasmuch as the air or other aeriform fluid thus admitted, acts as a barrier to the downflow into the retorts a of the fire gases, as is indicated by the arrows in Fig. 2, and this is effected without in any way interfering with the proper updraft through the stacks d.

It is important that the combustion chamber between the fire boxes or generators B and the retort-chamber should be sufficiently large to permit of practically complete combustion of the furnace gases before they enter the retort chamber. Furthermore, the distribution of the gases on their circuitous course through the horizontal flues should be capable of regulation, as, for instance, by fire-tile slides s which are capable of being operated from the exterior of the furnace so as to regulate the effective size of the openings and to direct the gases in the desired direction, as is the practice in the gasifying of coal in vertical retorts heated by horizontal flues. The temperature of the gases in the bottom of the retort-heating chamber or bench should be approximately 1500° C., and the fire gases should leave the chamber and enter the bottom of the shafts d at about 750° C.

The alunite to be calcined is screened to a convenient size, say one inch mesh. Any large amount of dust or fines should be removed. The ore is then fed into the hoppers and passes therefrom into the upper end of the shafts d. In starting the furnace, it is preferable to have each retort and shaft filled with ore that has previously been completely calcined. The products of combustion from the generators B should then be admitted into the retort-chamber and the temperature raised gradually until, as hereinbefore indicated, the temperature of the gases entering the shafts d is not less than 750° C. and those entering the retort-chamber at the bottom thereof not less than 1500° C. After these temperatures have continued for about one hour, and when the lower end of the vertical center of the charge of the retorts is not less than 900° C., the automatic rotating gates j are started. The rotation of the gates is continued until a sample of the alunite removed through the sampling tubes p at the bottom of the retorts just shows a faint trace of soluble alumina. The number of revolutions of the said automatic discharge gate should then be very

slightly decreased. It is contemplated to keep the discharge of the calcined alunite and the admission of the feed in such correspondence that the retorts will remain practically full during the operation.

Although I find it particularly convenient and desirable to employ upright or vertical retorts or muffles, for the calcining of the alunite, it will be understood that I do not restrict myself thereto, inasmuch as, in some instances, retorts or muffles other than those of the upright or vertical type may be used to advantage. It will also be understood that in using the expression "retort" or "muffle," throughout the specification, I use it in the generic sense, that is to say, as including a calcining chamber wherein the alunite is undergoing calcination and whose walls are heated externally by the fire gases.

The recovery of the sulfuric acid from the retorts or muffles is effected, as hereinbefore indicated, by withdrawing the gases through the exit pipes H, or the like, provided for the purpose, this withdrawal being effected by any suitable exhaust (not shown), familiar to the art. They are first, preferably, received in a suitable condenser or condensers wherein the sulfuric acid and SO<sub>3</sub> are recovered by condensation, or by condensation assisted by absorption, and the SO<sub>2</sub> is converted into sulfuric acid either by the lead chamber process or by the contact process, as the case may be. In fact, the particular manner of recovering the gases available as sulfuric acid may be appropriately varied to accommodate itself to the particular choice of the operator, the local market conditions, freight facilities, and the like, the process being sufficiently flexible to permit the necessary selection in this regard.

Having thus described my invention what I claim is:

1. The method of calcining alunite, which comprises dividing the calcining operation into two stages, in the first of which the alunite is traversed by furnace gases, and in the second of which the partly calcined alunite is heated from without, carrying off separately the gases evolved from the second stage of the calcining operation and recovering sulfuric acid therefrom; substantially as described.

2. The method of calcining alunite, which comprises dividing the calcining operation into two stages, in the first of which the operation is conducted at a final temperature of about 600° C., and in the second of which the calcining operation is completed at a final temperature ranging from 900° C. to 1000° C., and carrying off separately the gases evolved in the second stage of the calcining operation and recovering sulfuric acid therefrom; substantially as described.

3. The method of calcining alunite, which comprises dividing the calcining operation

into two stages, the partly calcined product from the first stage being progressively supplied to take the place of the fully calcined product withdrawn from the second stage, 5 and the gases evolved from the second stage of the operation being carried off separately from those evolved in the first stage thereof; substantially as described.

4. The method of calcining alunite, which 10 comprises dividing the calcining operation into two stages, in the first stage of which the alunite is traversed by furnace gases and in the second of which the partly calcined product from the first stage is heated from 15 without, the gases evolved from the second stage being carried off separately from those evolved in the first stage; substantially as described.

5. The method of calcining alunite, which 20 comprises subjecting an upright column of alunite to calcination, by fire gases applied externally to the lower portion of the column and admitted internally into the upper part of the column, thereby dividing the calcining operation into two stages, and carrying off separately gases evolved from the lower portion of the column; substantially as described.

6. The method of calcining alunite, which 30 comprises subjecting an upright column of alunite to calcination, by fire gases applied externally to the lower portion of the column and admitted internally into the upper part of the column, thereby dividing the calcining operation into two stages, maintaining 35 a draft for the fire gases through the upper part of the column, drawing off separately gases from the lower part of the column, and substantially neutralizing any 40 tendency for the fire gases to enter the lower part of the column by introducing below the point of entrance of the fire gases into the upper portion of the column an aeriform fluid under pressure; substantially as described.

45 7. The method of calcining alunite with the recovery of the sulfuric acid therefrom, which comprises dividing the calcining operation into two stages, in the first of which

the moisture and the water of composition 50 are substantially expelled from the alunite, and in the second of which the sulfuric anhydrid and the sulfuric acid evolved is recovered by condensation and absorption; substantially as described. 55

8. The method of calcining alunite with the recovery of sulfuric acid therefrom, which comprises dividing the calcining operation into two stages, in the first of which the moisture and the water of composition 60 are substantially expelled from the alunite, and in the second stage of which steam is admitted in such proportion as to convert a large part of the sulfurous anhydrid and sulfuric anhydrid into sulfuric acid and recovering the remainder of sulfuric anhydrid by condensation and absorption; substantially as described. 65

9. The method of calcining alunite with the recovery of sulfuric anhydrid and sulfuric acid, which comprises dividing the calcining operation into two stages, in the first of which the moisture and the water of composition are substantially expelled from the alunite, and in the second of which air is admitted in regulated quantity, and recovering the sulfuric anhydrid and acid by condensation and absorption; substantially as described. 75

10. The method of calcining alunite with the recovery of sulfuric anhydrid and sulfuric acid, which consists in dividing the calcining operation into two stages, in the first of which the moisture and water of composition are substantially expelled from 80 the alunite, and in the second of which steam and air are admitted in regulated quantity, and recovering the resulting sulfuric acid and the remnant sulfuric anhydrid by condensation and absorption; substantially as 85 described. 90

In testimony whereof I affix my signature, in presence of two witnesses.

HOWARD F. CHAPPELL.

Witnesses:

MARTIN M. BRASSEE,  
WALTER MANASSE.

Copies of this patent may be obtained for five cents each, by addressing the "Commissioner of Patents, Washington, D. C."